

March 27, 1951

E. MARBURG

2,546,270

TREATING BIG-END-DOWN INGOTS

Filed Feb. 13, 1948

FIG. 1.



FIG. 2.



FIG. 3.



INVENTOR:

EDGAR MARBURG,  
BY:  
John E. Jackson  
his Attorney.

## UNITED STATES PATENT OFFICE

2,546,270

## TREATING BIG-END-DOWN INGOTS

Edgar Marburg, Pittsburgh, Pa., assignor to  
United States Steel Company, a corporation of  
New Jersey

Application February 13, 1948, Serial No. 8,171

4 Claims. (Cl. 22—200)

1

This invention relates to a method of treating big-end-down ingots and is a continuation-in-part of my copending application, Serial No. 602,912, filed July 2, 1945, now abandoned.

In preparing steel for rolling, hot metal is poured into an ingot mold having a hot top for providing a sinkhead which will not complete freezing until the remainder of the ingot has frozen. After the metal has become sufficiently solidified, the mold is removed therefrom and the ingot is charged into the soaking pit. An ingot of normal size (18 to 25 inches per side) will freeze completely solid in 1 to 2½ hours' time if left in the mold. If exposed to air by stripping, the time will be somewhat less. In order to accomplish its purpose of providing a reservoir of liquid metal to prevent central pipe, the hot top sinkhead must be the last metal to freeze. If the ingot were allowed to freeze completely solid in the mold there would be no question about the sinkhead being the last metal allowed to freeze. However, it is uneconomical to hold all the ingots in their molds until completely solid and, therefore, they are normally removed from the mold while their centers are still liquid. The conventional hot tops now in use are removed from the ingot during or before stripping after which the liquid metal in the sinkhead, due to the smaller size of the latter and the thinner solidified wall formed therein will freeze at a faster rate than the ingot body. If the hot top is removed too soon after pouring, the sinkhead may then freeze before the ingot itself, and when the ingot finally freezes, a central cavity (secondary pipe) will develop due to the lack of feeder metal. It is necessary, therefore, to set a minimum time for ingots to be held at the platform so that when they are stripped, the freezing of the ingot body will be completed before that of the sinkhead. After the molds are stripped from the ingots and the latter are substantially solidified, they are charged into the soaking pits. Fire clay is the material commonly used to make hot tops and this material tends to fuse with hot metal, with the result that under the best conditions of stripping, fairly large portions of the hot top may remain adhering to the ingot when it is heated in the soaking pits and subsequently rolled. This clay may, and frequently does, cause damage to the surface of the rolls or ingots during rolling. If it becomes mixed with the mill scale, it comprises a very undesirable component of the scale, which is recovered and charged into the blast furnace.

The patent to Kenney, No. 1,137,144, discloses a hot top which is retained on the ingot after stripping, but it also remains on the ingot in the soaking pit. This obstructs the passage of the heat into the hot top during the heating of the ingot and will cause damage to the surface of the steel being rolled and to the roll surfaces, as well as contaminating the scale.

2

It is an object of my invention to provide a method of treating big-end-down ingots in which the mold is stripped as soon as practicable from the ingot, but the hot top is retained in place until the ingot has substantially solidified and then removed prior to charging the ingot into the soaking pit.

A further object is to provide a method of treating big-end-down ingots which will increase the life of the ingot mold by reducing the length of time ingots must be held at the pouring platform before stripping.

A still further object is to provide a method of treating big-end-down ingots whereby the time between pouring and charging is decreased, thus charging ingots at a higher temperature, shortening heating times, reducing fuel costs, and improving the quality of product by reducing scaling of ingot surfaces.

Another object is to provide such a method that can be carried out without the use of special equipment.

These and other objects will be more apparent after referring to the following specification and attached drawings, in which:

Figure 1 is a top plan view of the hot top in place on a mold;

Figure 2 is a sectional view on the line II—II of Figure 1; and

Figure 3 is a sectional view on the line III—III of Figure 2.

My method of treating the ingots comprises placing a hot top on a big-end-down mold, pouring the hot metal into the mold, stripping the mold from the ingot while retaining the hot top in place on the ingot, permitting the ingot to stand with the hot top in place until the ingot has substantially solidified, and finally removing the hot top before charging into the soaking pit. The hot top used is preferably a sectional coke hot top as disclosed in the drawings.

Referring more particularly to the drawings, reference numeral 2 represents the top of a rectangular big-end-down mold. The hot top consists of two side slabs 4 and two end slabs 6 between the ends of the side slabs and the mold. The side slabs have their lower edges bevelled at 8, the outside faces of the bevelled portion being of the same contour as the interior of the mold, the remaining portion of the outside and the entire interior surfaces being flat. The bottom of the side slabs are substantially wider than the top in order to form a wedge surface on each end of the slab. Slots 10 are provided in the side slabs 4 for the insertion of support hooks 12 which are preformed with a hook portion 14 having a slightly smaller angle than the slot so that when inserted as shown, the hooks will remain rigidly attached to the slab. The hooks are supported on top of the mold as shown, and the outer portion of each hook is flared at 16 to permit ready placing thereof over the top of the mold. Clear-

ance 17 is provided between the wire hook and the mold to allow for scrap or rough edges thereon. By locating slots 10 below the centers of the slabs, the weight of the overhanging top portion causes the bevelled lower portion to contact the mold closely. Further, the support hook wire has ample clearance and causes no separation between mold and hot top, as it would if the hook were placed under the bottom of the slab. The end slabs 6 have a bevelled lower edge 18 similar to the bevelled lower edge 8, but the tops and bottoms of these slabs are of substantially the same width, slightly less than the width of the mold, and no wedge surface is formed on the edges.

In assembling the hot top on the mold, a pair of hooks 12 are placed in the openings 10 of each side slab 4 and the slabs placed in position and supported from the top of the mold, as shown, with their lower bevelled faces in contact with the mold. The end slabs 6 are then wedged in place with their outer lower faces in contact with the mold wall and their inner flat faces in contact with the wedge end surfaces of the side slabs 4. This locks the hot top in place and prevents it from floating as the metal rises therein. The joints remain closed during pouring without binding wire or other fastening, because the outward pressure of the steel against the lower part of the slabs is greater than its outward pressure against the top of the slabs. The bevelled lower edges contact the mold for a sufficient distance to prevent metal rising between the mold and the slabs.

In order to insure that the slabs remain on the ingot after the mold is stripped therefrom, the slabs may be provided with openings 20 in their inner surfaces into which the hot metal flows, although we have found that the slabs will generally remain on the ingots without these slots. During stripping the wire hooks 12 are bent upwardly by the mold without pulling the slabs from the ingot.

While the hot top described above is particularly adapted for performing my method, other types of hot tops may also be used as long as they are easily removed from the ingot prior to charging into the soaking pit. The slabs are preferably made of coke or limestone, since these materials do not stick to the mold in the same manner as fire clay. Also, these materials are less harmful to soaking pit bottoms and less likely to damage the roll or ingot surfaces during rolling. However, clay hot tops, while not as satisfactory as coke or limestone, may be used if their inside surfaces are coated with a suitable material for preventing sticking of the clay to the metal. The hot top shown may be easily removed by the soaking pit crane lifting tongs, especially if made of coke or limestone.

In summary then, my method consists of:

- (1) Placing a hot top on a big-end-down mold;
- (2) Pouring the hot metal into the mold;
- (3) Stripping the mold from the ingot a relatively short time after pouring. The length of time the mold must remain on the ingot will vary with the size of the ingot, but in most instances, the ingot will have solidified sufficiently to enable the mold to be removed after a period of from 15 to 45 minutes;
- (4) Permitting the ingot to stand with the hot top in place until the ingot has substantially solidified; and
- (5) Removing the hot top from the ingot before charging it into the soaking pit.

My improved method permits stripping the molds much sooner after pouring than at present, thus resulting in longer mold life, fewer molds required because of more frequent use of the molds, and quicker delivery of the ingots to the soaking pit. The reheating time of the ingots is also reduced and a clean ingot is delivered to the rolling mill. Further, my method does not involve the use of any additional equipment and the flow of the ingot from the pouring floor to the soaking pit is essentially the same as in usual practice.

While one embodiment of my invention has been shown and described, it will be apparent that other adaptations and modifications may be made without departing from the scope of the following claims.

I claim:

1. A method of treating big-end-down ingots which comprises placing a hot top on a mold, pouring hot metal into the mold, completely stripping the mold from the ingot between approximately 15 and 45 minutes after pouring while retaining the hot top in place on the ingot, permitting the ingot to stand with the hot top in place until the ingot has substantially solidified, removing the hot top and then charging the ingot into the soaking pit.

2. A method of treating big-end-down ingots which comprises placing a sectional hot top on a mold, pouring hot metal into the mold, completely stripping the mold from the ingot between approximately 15 and 45 minutes after pouring while retaining the hot top in place on the ingot, permitting the ingot to stand with the hot top in place until the ingot has substantially solidified, removing the hot top and then charging the ingot into the soaking pit.

3. A method of treating big-end-down ingots which comprises placing a coke hot top on a mold, pouring hot metal into the mold, completely stripping the mold from the ingot between approximately 15 and 45 minutes after pouring while retaining the hot top in place on the ingot, permitting the ingot to stand with the hot top in place until the ingot has substantially solidified, removing the hot top and then charging the ingot into the soaking pit.

4. A method of treating big-end-down ingots which comprises placing a sectional coke hot top on a mold, pouring hot metal into the mold, completely stripping the mold from the ingot between approximately 15 and 45 minutes after pouring while retaining the hot top in place on the ingot, permitting the ingot to stand with the hot top in place until the ingot has substantially solidified, removing the hot top and then charging the ingot into the soaking pit.

#### REFERENCES CITED

The following references are of record in the file of this patent:

#### UNITED STATES PATENTS

|    | Number    | Name     | Date          |
|----|-----------|----------|---------------|
| 60 | 1,137,144 | Kenney   | Apr. 27, 1915 |
|    | 1,737,665 | Messler  | Dec. 3, 1929  |
| 70 | 1,978,996 | Gathmann | Oct. 30, 1934 |
|    | 2,075,039 | Kauffman | Mar. 30, 1937 |
|    | 2,102,258 | Dornin   | Dec. 14, 1937 |
|    | 2,433,775 | Marburg  | Dec. 30, 1947 |
|    | 2,444,838 | Marburg  | July 6, 1948  |